

## UNITED STATES PATENT OFFICE

2,080,159

## PROCESS OF TREATING STEEL

Robert S. Archer, Chicago, Ill., assignor to The Republic Steel Corporation, Youngstown, Ohio, a corporation of New Jersey

No Drawing. Application June 5, 1935, Serial No. 25,127. Renewed March 10, 1937

3 Claims. (Cl. 22—214)

This invention relates to the art of treating metals, and particularly to a method of preventing the formation of so-called "hair line seams" in steel articles.

5 Certain steels, as made by ordinary methods, contain so-called "hair line seams". These "seams" are not seams in the sense of crevices, but are bodies of non-metallic material occluded in the steel. Usually these "seams" are parallel, 10 to and just below the surface of rolled steel articles. They are usually in the form of elongated bodies of small thickness, much like hairs. It is quite difficult to detect such "seams" by any of the usual laboratory apparatus, including a microscope, but they can be located by machining the steel article parallel to its long axis. In such cases, they appear as lines resembling cracks of hair line thickness in the machined surface. For example, if a round rolled bar containing these 15 "seams" is centered in a lathe, rotated about its long axis and the surface layer is machined off, the axially extending "seams" in the machined surface can be detected. Deeper seated "seams" may similarly be located by taking further cuts off the bar. Generally speaking, most of such 20 "seams" are found in the article just below the surface, but often some are found at greater depths below the surface. These "hair line seams" are quite objectionable in steel articles intended for certain uses and render such articles 25 unsatisfactory if present in excess of certain small amounts.

I have discovered that the "hair line seams" are more often encountered in steels which contain 30 ingredients which, under ordinary treating and casting conditions, tend to form in the steel non-metallic substances of higher fusing point than that of the steel. For example, these "seams" are common under prior, standard, steel making 35 practices, in steels of the SAE 2345 type which have the following general composition:

|           |              |
|-----------|--------------|
| Carbon    | .40 to .50   |
| Manganese | .60 to .70   |
| Phos      | .040 max.    |
| 45 Sul    | .050 max.    |
| Nickel    | 3.25 to 3.75 |

These steels, as well as others in the SAE 2300 series, and other steels including steels of the 50 SAE 1000 series, which contain between about .30% and about 1.00% of manganese with usual amounts of phosphorus and sulphur, may be treated by the method of this invention with success as measured by decrease in the number of 55 such "seams" as compared with similar untreated

steels. I believe that my method may be employed advantageously on a wide range of steels wherein there exists any tendency to formation of "hair line seams". It seems probable that the high melting point non-metallic substances which 5 form these "seams" are equiaxed inclusions in the ingot but are elongated into hairlike shape by the rolling operations.

I have discovered that the "hair line seams" may be greatly reduced in number and often 10 avoided completely by casting the steel in a protective and reactive atmosphere consisting largely or wholly of chlorine or a chlorine rich gas. I would prefer to use chlorine as such but, in order to maintain proper working conditions around 15 the molds, can and do, use less toxic chlorine compounds such as carbontetrachloride.

Altho I have mentioned chlorine and carbontetrachloride, these are not the only substances which can be used. In general, any chlorine containing compound which will decompose under 20 the temperatures present in the mold during casting and will liberate chlorine in adequate amounts for the intended purpose may be used. I believe that whatever carbon or hydrogen may be present in the chlorine compound which is used is unnecessary in bringing about the desired results and, as stated above, would prefer to use chlorine gas except that it tends to make unsatisfactory the working conditions about the molds.

I believe that the "hair line seams" are caused 30 by the presence of oxidized deoxidizers in the steel. Ordinarily, deoxidizers, such as small amounts of manganese, silicon, aluminum, zirconium or the like are added to the steel in the furnace, in the ladle or in the mold. These substances oxidize more or less completely and their oxides may remain entrapped in the steel. They 35 may react with other non-metallic substances to form complex compounds. Many of these oxides or substances or compounds are relatively infusible. Where aluminum is the deoxidizer used, the amount is small, ranging usually from about  $\frac{1}{2}$  pound to perhaps 2 pounds per ton of steel. The amounts of manganese, zirconium and silicon may be somewhat larger. "Hair line seams" have been found in steel of the SAE 2345 type to which between  $\frac{1}{2}$  pound and 1 pound of aluminum per ton had been added as a deoxidizer and in which substantially all the aluminum had 45 been oxidized. Treatment of similar steel by the present process has greatly reduced the number of "hair line seams".

In practicing the present process in a preferred manner, I tap the molten steel into a ladle and 50

add the usual amounts of metallic deoxidizer. Then I drop, pour in a small stream, or otherwise suitably introduce, liquid carbontetrachloride into a mold, for example, an ingot mold, just before, 5 and also during, pouring of the molten steel into the mold. Between about two pounds and about four pounds of this liquid for each 21" duodecagon mold making a 7500 pound ingot is sufficient for the desired results. This liquid vapor- 10 izes at once and being heavier than air tends to expel some of the air and dilute the remainder, particularly at the surface of the pool of metal in the mold and to a greater or lesser extent around the flowing stream of steel.

15 Two to four pounds of carbontetrachloride per 7500 pounds of steel is roughly  $\frac{1}{2}$  to 1 pound per ton of steel. Good results have been obtained with as little as about  $\frac{1}{4}$  pound per ton and also with more than  $1\frac{1}{2}$  pounds of carbontetrachloride 20 per ton of steel.

The foregoing treatment gives unexpected results. Considerable quantities of oxides collect in the form of lumps on the tops of ingots. No such collection of lumps occurs during the ordinary pouring of the same kind of steel. Collection of oxides in lump form as a result of the present process is believed to be due to some physical or chemical change in the oxides in the metal which is brought about by the foregoing 25 treatment. Chemical analysis made of these lumps has given the following ingredients and percentages thereof:—

|                                | Percent |
|--------------------------------|---------|
| FeO                            | 4.5     |
| MnO                            | 14.11   |
| SiO <sub>2</sub>               | 12.10   |
| Al <sub>2</sub> O <sub>3</sub> | 51.0    |
| CaO                            | 1.15    |
| Cl <sub>2</sub>                | 2.0     |
| 40 MgO                         | Trace   |

It seems probable that these lumps are collections of the dispersed substances which cause hair line seams, for chemical analyses of foreign material found in such seams shows between about 45 50% and about 80% of Al<sub>2</sub>O<sub>3</sub> and between about 20% and about 45% of SiO<sub>2</sub> by methods of analysis in which the oxides of iron, manganese and calcium were removed before determination of 50 Al<sub>2</sub>O<sub>3</sub> and SiO<sub>2</sub>.

Whatever may be the action which takes place by reason of the present process, the unexpected and practical result is that the number and size of hair line seams is greatly reduced, if not more or less completely eliminated, and quantities of 5 foreign material otherwise found in hair line seams collects in the form of lumps on the surface of the ingot.

It will be understood that the time when the metallic deoxidizer is added to the steel is not 10 critical on the present process. For example, the deoxidizer may be added in the furnace or in the mold and improved results, as regards decrease in the number of "seams" may be obtained.

I have thus described my invention in detail 15 so that others skilled in the art may understand and be able to practice the same, but not for the purpose of defining the scope of my invention. The scope is defined in what is claimed.

What is claimed is:

1. The method of treating steel to prevent the formation of "hair line seams" in articles rolled from such steel, which includes the steps of adding to molten steel a small amount of a metallic deoxidizer and bringing such steel into a mold 25 containing carbon tetrachloride, a chlorine rich atmosphere, thereby collecting and bringing to the top surface of the steel "seam causing" oxides.

2. The method of treating steel to prevent the formation of "hair line seams" in articles rolled 30 from such steel which includes the steps of making molten steel containing between about .30% and about 1.00% of manganese, adding thereto a small amount of a metallic deoxidizer, and collecting oxidized deoxidizers by bringing such steel 35 into a mold together with between about  $\frac{1}{4}$  pound and about  $1\frac{1}{2}$  pounds of carbontetrachloride per ton of steel, part of the carbon tetrachloride being placed in the mold before the steel enters the mold.

3. The method of treating steel which includes the steps of adding a small amount of metallic deoxidizer to molten steel containing manganese and collecting non-metallic oxides in the form of lumps on the top surface of the steel by pouring such steel into a mold and bringing into the mold shortly prior to and during such pouring between about one-quarter pound and one and one-half pounds of carbon tetrachloride per ton of steel.

ROBERT S. ARCHER. 50

#### CERTIFICATE OF CORRECTION.

Patent No. 2,080,159.

May 11, 1937.

ROBERT S. ARCHER.

It is hereby certified that error appears in the printed specification of the above numbered patent requiring correction as follows: Page 1, first column, line 43, for ".50" read .90; and page 2, second column, line 26, claim 1, strike out the words "carbon tetrachloride"; and that the said Letters Patent should be read with these corrections therein that the same may conform to the record of the case in the Patent Office.

Signed and sealed this 29th day of June, A. D. 1937.

Henry Van Arsdale

Acting Commissioner of Patents.

(Seal)

add the usual amounts of metallic deoxidizer. Then I drop, pour in a small stream, or otherwise suitably introduce, liquid carbontetrachloride into a mold, for example, an ingot mold, just before, 5 and also during, pouring of the molten steel into the mold. Between about two pounds and about four pounds of this liquid for each 21" duodecagon mold making a 7500 pound ingot is sufficient for the desired results. This liquid vapor- 10 izes at once and being heavier than air tends to expel some of the air and dilute the remainder, particularly at the surface of the pool of metal in the mold and to a greater or lesser extent around the flowing stream of steel.

15 Two to four pounds of carbontetrachloride per 7500 pounds of steel is roughly  $\frac{1}{2}$  to 1 pound per ton of steel. Good results have been obtained with as little as about  $\frac{1}{4}$  pound per ton and also with more than  $1\frac{1}{2}$  pounds of carbontetrachloride 20 per ton of steel.

The foregoing treatment gives unexpected results. Considerable quantities of oxides collect in the form of lumps on the tops of ingots. No such collection of lumps occurs during the ordinary pouring of the same kind of steel. Collection of oxides in lump form as a result of the present process is believed to be due to some physical or chemical change in the oxides in the metal which is brought about by the foregoing 25 treatment. Chemical analysis made of these lumps has given the following ingredients and percentages thereof:—

|                                | Percent |
|--------------------------------|---------|
| FeO                            | 4.5     |
| MnO                            | 14.11   |
| SiO <sub>2</sub>               | 12.10   |
| Al <sub>2</sub> O <sub>3</sub> | 51.0    |
| CaO                            | 1.15    |
| Cl <sub>2</sub>                | 2.0     |
| 40 MgO                         | Trace   |

It seems probable that these lumps are collections of the dispersed substances which cause hair line seams, for chemical analyses of foreign material found in such seams shows between about 45 50% and about 80% of Al<sub>2</sub>O<sub>3</sub> and between about 20% and about 45% of SiO<sub>2</sub> by methods of analysis in which the oxides of iron, manganese and calcium were removed before determination of 50 Al<sub>2</sub>O<sub>3</sub> and SiO<sub>2</sub>.

Whatever may be the action which takes place by reason of the present process, the unexpected and practical result is that the number and size of hair line seams is greatly reduced, if not more or less completely eliminated, and quantities of 5 foreign material otherwise found in hair line seams collects in the form of lumps on the surface of the ingot.

It will be understood that the time when the metallic deoxidizer is added to the steel is not 10 critical on the present process. For example, the deoxidizer may be added in the furnace or in the mold and improved results, as regards decrease in the number of "seams" may be obtained.

I have thus described my invention in detail 15 so that others skilled in the art may understand and be able to practice the same, but not for the purpose of defining the scope of my invention. The scope is defined in what is claimed.

What is claimed is:

1. The method of treating steel to prevent the formation of "hair line seams" in articles rolled from such steel, which includes the steps of adding to molten steel a small amount of a metallic deoxidizer and bringing such steel into a mold 25 containing carbon tetrachloride, a chlorine rich atmosphere, thereby collecting and bringing to the top surface of the steel "seam causing" oxides.

2. The method of treating steel to prevent the formation of "hair line seams" in articles rolled 30 from such steel which includes the steps of making molten steel containing between about .30% and about 1.00% of manganese, adding thereto a small amount of a metallic deoxidizer, and collecting oxidized deoxidizers by bringing such steel 35 into a mold together with between about  $\frac{1}{4}$  pound and about  $1\frac{1}{2}$  pounds of carbontetrachloride per ton of steel, part of the carbon tetrachloride being placed in the mold before the steel enters the mold.

3. The method of treating steel which includes the steps of adding a small amount of metallic deoxidizer to molten steel containing manganese and collecting non-metallic oxides in the form of lumps on the top surface of the steel by pouring such steel into a mold and bringing into the mold shortly prior to and during such pouring between about one-quarter pound and one and one-half pounds of carbon tetrachloride per ton of steel.

ROBERT S. ARCHER. 50

#### CERTIFICATE OF CORRECTION.

Patent No. 2,080,159.

May 11, 1937.

ROBERT S. ARCHER.

It is hereby certified that error appears in the printed specification of the above numbered patent requiring correction as follows: Page 1, first column, line 43, for ".50" read .90; and page 2, second column, line 26, claim 1, strike out the words "carbon tetrachloride"; and that the said Letters Patent should be read with these corrections therein that the same may conform to the record of the case in the Patent Office.

Signed and sealed this 29th day of June, A. D. 1937.

Henry Van Arsdale

Acting Commissioner of Patents.

(Seal)

CERTIFICATE OF CORRECTION.

Patent No. 2,080,159.

May 11, 1937.

ROBERT S. ARCHER.

It is hereby certified that error appears in the printed specification of the above numbered patent requiring correction as follows: Page 1, first column, line 43, for ".50" read .90; and page 2, second column, line 26, claim 1, strike out the words "carbon tetrachloride"; and that the said Letters Patent should be read with these corrections therein that the same may conform to the record of the case in the Patent Office.

Signed and sealed this 29th day of June, A. D. 1937.

Henry Van Arsdale

(Seal)

Acting ~~Commissioner~~ of Patents.